# EUROPEAN PATENT SPECIFICATION

(11) **EP 1 496 331 B1**
(45) Date of publication and mention of the grant of the patent: **05.11.2008**
(21) Application number: 04024471.7
(22) Date of filing: 10.08.1999
(51) Int. Cl.: F41H 5/04

(54) **Hybrid protective composite**
Hybrides Schutzkomposit
Composite hybride de protection

(30) Priority: 21.12.1998 US 217360
(43) Date of publication of application: 12.01.2005
(62) Divisional of application: 99942041.7
(73) Proprietor: E.I. DU PONT DE NEMOURS AND COMPANY, Wilmington, DE 19898 (US)
(72) Inventor: Chiou, Minshon J., Chesterfield, VA 23838 (US)
(74) Representative: Beacham, Annabel Rose

(56) References cited:
- WO-A-91/06821
- WO-A-93/00564
- WO-A-93/11290
- WO-A-93/20400
- WO-A-94/14023
- WO-A-96/32621
- WO-A-97/49849
- WO-A-98/05917
- WO-A-98/17136
- WO-A-99/47880
- GB-A- 2 198 628
- US-A- 5 578 358

## Description

### BACKGROUND OF THE INVENTION

### Field of the Invention -

This invention relates to protective composites in the field of knife and ice pick stab resistance which composites provide, on one hand, greater protection for a given weight; and, on the other hand, equivalent protection in a lighter weight, in comparison with other protective composites currently available. The composite of this invention is flexible.

### Description of the Prior Art -

International Publication WO 93/20400, published 14 October 1993, discloses the use of polybenzoxazole and polybenzothiazole fibers in ballistic resistant articles.

United States Patent No. 5,578,358, issued November 26, 1996, on the application of Foy et al. discloses a penetration-resistant structure made from woven aramid yarns having particularly low linear density.

International Publication No. WO 93/00564, published January 7, 1993, discloses ballistic structures using layers of fabric woven from high tenacity para-aramid yarn.

United States Patent No. 5,472,769, issued December 5, 1995, as an example of attempts to provide both puncture resistance and ballistic resistance, describes a combination of knitted aramid yarn layers and deflection layers of materials such as metal wire.

European Patent Application No. 670,466, published September 6, 1995, describes a ballistic and stab-resistant system wherein the knife stab resistance is imparted by embedding chainmail in a polymer resin.

International Publication No. WO 98/05917, which forms a starting point for claim 1, discloses a puncture resistant garment comprising a ballistic resistant layer and a knife and ice pick resistant layer containing a plurality of tightly-woven penetration resistant fabrics.

UK Patent No. GB 2 198 628 discloses the use of polybenzothiazole fibres in textile armour for protection against projectile fragments comprising a plurality of textile layers.

### SUMMARY OF THE INVENTION

The present invention provides a protective composite structure with a plurality of primarily knife resistant layers of woven fabric comprising polybenzoxale (PBO) or polybenzothiazole (PBT) fibers, and a plurality of primarily ice pick resistant layers of tightly-woven penetration resistant fabric having a tightness factor of at least 0.75.

### BRIEF DESCRIPTION OF THE DRAWINGS

The Fig. shows an expanded perspective view of a composite of this invention.

### DETAILED DESCRIPTION

Improvements in composites for knife and ice pick stab protection are continually sought, although often as a secondary quality after ballistic protection. Generally, knife and ice pick stab protection is required in garments worn by guards, police officers, and the like; and ballistic protection is, also, a desirable quality in such garments. Such garments must be as flexible as possible to ensure comfort sufficient that the garment will be readily worn.

While the kernel of the present invention resides in use of a particular combination of two different layers of materials to afford the desired protection results, each of the different layers do exhibit a primary utility in the combination.

The materials of this hybrid composite which are primarily effective for the knife stab resistance are polybenzoxazole or polybenzothiazole in fiber form in woven layers.

Polybenzoxazole and polybenzothiazole are generally, as described in the aforementioned WO 93/20400, incorporated herein by reference. Polybenzoxazole and polybenzothiazole are preferably made up of mers of the following structures:

While the aromatic groups shown joined to the nitrogen atoms may be heterocyclic, they are preferably carbocyclic; and while they may be fused or unfused polycyclic systems, they are preferably single six-membered rings. While the group shown in the main chain of the bis-azoles is the preferred para-phenylene group, that group may be replaced by any divalent organic group which doesn't interfere with preparation of the polymer, or no group at all. For example, that group may be aliphatic up to twelve carbon atoms, tolylene, biphenylene, bis-phenylene ether, and the like.

The polybenzoxazole and polybenzothiazole used to make fibers of this invention should have at least 25 and preferably at least 100 mer units. Preparation of the polymers and spinning of those polymers is disclosed in the aforementioned International Publication WO 93/20400.

The polybenzoxazole and polybenzothiazole fibers are woven in any, generally-used, fabric configuration such as plain weave, crowfoot weave, basket weave, satin weave, and the like. Plain weave is preferred.

It is believed that fibers and yarns of any linear density will be effective to increase knife stab resistance in the present invention. The preferred linear density for individual fibers should be 0.3 to 17 dtex, and 0.5 to 3.5 dtex is most preferred. Yarns in the range of 100 to 3300 dtex are preferred with 220 to 1700 dtex being most preferred. Yarns with a linear density of greater than 3300 dtex are generally more difficult to produce and use efficiently and yarns with a linear density of less than 100 dtex are difficult to weave without damage to the yarn.

The materials of this hybrid composite which are primarily effective for the ice pick stab resistance can be, among other things, polyamide and polyolefin; and can, also, be polybenzoxazole and polybenzothiazole.

When the other polymer is polyamide, aramid is preferred. By "aramid" is meant a polyamide wherein at least 85% of the amide (-CO-NH-) linkages are attached directly to two aromatic rings. Suitable aramid fibers are described in Man-Made Fibers - Science and Technology, Volume 2, Section titled Fiber-Forming Aromatic Polyamides, page 297, W. Black et al., Interscience Publishers, 1968. Aramid fibers are, also, disclosed in U.S. Patents 4,172,938; 3,869,429; 3,819,587; 3,673,143; 3,354,127; and 3,094,511.

Additives can be used with the aramid and it has been found that up to as much as 10 percent, by weight, of other polymeric material can be blended with the aramid or that copolymers can be used having as much as 10 percent of other diamine substituted for the diamine of the aramid or as much as 10 percent of other diacid chloride substituted for the diacid chloride or the aramid.

The preferred aramid is a para-aramid and poly(p-phenylene terephthalamide) (PPD-T) is the preferred para-aramid. By PPD-T is meant the homopolymer resulting from mole-for-mole polymerization of p-phenylene diamine and terephthaloyl chloride and, also, copolymers resulting from incorporation of small amounts of other diamines with the p-phenylene diamine and of small amounts of other diacid chlorides with the terephthaloyl chloride. As a general rule, other diamines and other diacid chlorides can be used in amounts up to as much as about 10 mole percent of the p-phenylene diamine or the terephthaloyl chloride, or perhaps slightly higher, provided only that the other diamines and diacid chlorides have no reactive groups which interfere with the polymerization reaction. PPD-T, also, means copolymers resulting from incorporation of other aromatic diamines and other aromatic diacid chlorides such as, for example, 2,6-naphthaloyl chloride or chloro- or dichloroterephthaloyl chloride or 3,4'-diaminodiphenylether.

When the other polymer is polyolefin, polyethylene or polypropylene are preferred. By polyethylene is meant a predominantly linear polyethylene material of preferably more than one million molecular weight that may contain minor amounts of chain branching or comonomers not exceeding 5 modifying units per 100 main chain carbon atoms, and that may also contain admixed therewith not more than about 50 weight percent of one or more polymeric additives such as alkene-1-polymers, in particular low density polyethylene, propylene, and the like, or low molecular weight additives such as anti-oxidants, lubricants, ultra-violet screening agents, colorants and the like which are commonly incorporated. Such is commonly known as extended chain polyethylene (ECPE). Similarly, polypropylene is a predominantly linear polypropylene material of preferably more than one million molecular weight. High molecular weight linear polyolefin fibers are commercially available. Preparation of polyolefin fibers is discussed in US 4,457,985.

As a general rule, flexible articles with ice pick penetration resistance are made using layers of fabric woven from yarn material with high tenacity and toughness; and the degree of ice pick penetration resistance is, among other things, a function of the linear density of the yarn and tightness of the weave. The lower the linear density of the yarn and the tighter the weave, the greater the ice pick penetration resistance.

"Fabric tightness factor" and "Cover factor" are names given to the density of the weave of a fabric. Cover factor is a calculated value relating to the geometry of the weave and indicating the percentage of the gross surface area of a fabric which is covered by yarns of the fabric. The equation used to calculate cover factor is as follows (from Weaving: Conversion of Yarns to Fabric, Lord and Mohamed, published by Merrow (1982), pages 141-143):
d_{w} = width of warp yarn in the fabric
d_{f} = width of fill yarn in the fabric
P_{w} = pitch of warp yarns (ends per unit length)
p_{f} = pitch of fill yarns
   ${C}_{w} = \frac{{d}_{w}}{{p}_{w}} {C}_{f} = \frac{{d}_{f}}{{p}_{f}}$ $Fabric Cover Factor = {C}_{fab} = \frac{total area obscured}{area enclosed}$ $\begin{matrix}{C}_{fab} & = \frac{\left({p}_{w}-{d}_{w}\right) ⁢ {d}_{f} + {d}_{w} ⁢ {p}_{f}}{{p}_{w} ⁢ {p}_{f}} \\ & = \left({C}_{f}+{C}_{w}-{C}_{f}⁢{C}_{w}\right)\end{matrix}$
   Depending on the kind of weave of a fabric, the maximum cover factor may be quite low even though the yarns of the fabric are situated close together. For that reason, a more useful indicator of weave tightness is called the "fabric tightness factor". The fabric tightness factor is a measure of the tightness of a fabric weave compared with the maximum weave tightness as a function of the cover factor. $Fabric tightness factor = \frac{actual cover factor}{maximum cover factor}$

For example, the maximum cover factor which is possible for a plain weave fabric is 0.75; and a plain weave fabric with an actual cover factor of 0.68 will, therefore, have a fabric tightness factor of 0.91. The preferred weave for practice of this invention is plain weave.

The particular combination of this invention, utilizing special penetration resistant materials, exhibits an ice pick and knife penetration resistance which is much greater than would be expected from the sum of the penetration resistance of the individual elements of the combination. The individual elements in the combination of this invention have a particular element-to-element relationship.

The primarily knife penetration resistant layers of polybenzoxazole or polybenzothiazole fabric may be located anywhere in the composite of this invention. Generally, more than one layer of these fabrics will be required to afford the desired knife stab protection. Each layer of polybenzoxazole and polybenzothiazole generally has an areal density of 75 to 450 grams per square meter and, generally, 1 to 15 layers are used. The areal density of the layers depends greatly on the form of the network and on the kind and linear density of the fibers. Generally, however, the polybenzoxazole and polybenzothiazole fibers constitute from 10 to 90, and preferably 15 to 50, weight percent of the total composite.

The primarily ice pick stab resistant fabric layers are made from tightly-woven yarns of high strength fibers wherein the yarns generally have a linear density of less than 500 dtex and, preferably, the individual fibers in those yarns have a linear density of 0.2 to 2.5 dtex and more preferably 0.7 to 1.7 dtex. These layers can be made from polyamides, polyolefins, polybenzoxazoles, polybenzothiazole, or other fibers usually used for penetration resistance. The preferred material for these layers is para-aramid yarns. The preferred linear density for the yarns is 100 to 500 dtex and those yarns are preferably woven to a fabric tightness factor of 0.75 to 1.00 or, perhaps, higher, and, more preferably greater than 0.95. It is most preferred that the tightly woven fabric layers have a relationship between the yarn linear density (dtex) and the fabric tightness factor as follows:

Y > X 6.25 X 10⁻⁴ + 0.69 wherein, Y = fabric tightness factor and X = yarn linear density, as disclosed in the aforementioned U.S. Patent No. 5,578,358.

Yarns used in any of the fabric layers of this invention should exhibit a tenacity of greater than 20 grams per dtex and as much as 50 grams per dtex or more; an elongation to break of at least 2.0% and as much as 6% or more; and a modulus of at least 270 grams per dtex and as much as 2000 grams per dtex or more.

A combination of the two elements of this invention is made by placing the two together, in face to face relation, with other layer materials therebetween or not, as desired. Other layer materials which may be placed among the two elements include, for example, water proofing materials, anti-trauma materials, and the like.

Improved ice pick and knife penetration resistance can be obtained using the two elements in accordance with this invention. A combination of the plurality of layers of woven polybenzoxazole or polybenzothiazole fibers and the plurality of tightly-woven penetration resistant layers, in accordance with the present invention, produces ice pick and knife penetration resistances which are much greater than the sum of those penetration resistances which would be exhibited by the elements taken individually.

The layers which form the sections of this composite can be joined such as by being sewn together or they can be stacked together and held, for example, in a fabric envelope. The layers which constitute each section are usually placed together and the composite can, thereby, be seen as a structure having distinct sections of layers.

The high knife penetration resistance of this invention is provided by the polybenzoxazole or polybenzothiazole fabric layers. The polybenzoxazole or polybenzothiazole fabric layers can be located anywhere in the article. The high ice pick penetration resistance of this invention is provided by the tightly woven fabric layers.

The Fig. shows the protective composite 10 of this invention with a section 11 of layers 12 of woven polybenzoxazole or polybenzothiazole, and a section 13 of layers 14 of tightly-woven layers. The layers 12 and 14 can be intermixed in any sequence such that sections 11 and 13 are not distinct.

### TEST METHODS

Linear Density. The linear density of a yarn is determined by weighing a known length of the yarn. "dtex" is defined as the weight, in grams, of 10,000 meters of the yarn.

In actual practice, the measured dtex of a yarn sample, test conditions, and sample identification are fed into a computer before the start of a test; the computer records the load-elongation curve of the yarn as it is broken and then calculates the properties.

Tensile Properties. Yarns tested for tensile properties are, first, conditioned and, then, twisted to a twist multiplier of 1.1. The twist multiplier (TM) of a yarn is defined as: $TM = \left(turns/cm\right) {\left(dtex\right)}^{1 / 2} / 30.3$

The yarns to be tested are conditioned at 25°C, 55% relative humidity for a minimum of 14 hours and the tensile tests are conducted at those conditions. Tenacity (breaking tenacity), elongation to break, and modulus are determined by breaking test yarns on an Instron tester (Instron Engineering Corp., Canton, Mass.).

Tenacity, elongation, and initial modulus, as defined in ASTM D2101-1985, are determined using yarn gage lengths of 25.4 cm and an elongation rate of 50% strain/minute. The modulus is calculated from the slope of the stress-strain curve at 1% strain and is equal to the stress in grams at 1% strain (absolute) times 100, divided by the test yarn linear density.

Penetration Resistance. Knife penetration resistance is determined on a sample to be tested using a boning knife (made by Russell Harrington Cutlery, Inc., Southbridge, Massachusetts, U.S.A.) with a single edged blade 15 cm (6 inches) long and about 2 cm (0.8 inch) wide, tapering toward the tip and having a Rockwell hardness of C-55. The tests are conducted in accordance with HPW test TP-0400.03 (28 November 1994) from H. P. White Lab., Inc. The test samples, placed on a 10% gelatin backing, are impacted with the knife, weighted to 4.55 kilograms (10 pounds) and dropped from various heights until penetration of the sample of greater than 6mm under test conditions is accomplished. Ice pick penetration is determined using the same procedure as set out above except that the boning knife is replaced with an ice pick 18 centimeters (7 inches) long and 0.64 centimeters (0.25 inch) in shaft diameter having a Rockwell hardness of C-42. Results are reported as penetration energy (joules) by multiplying kilogram-meters, from the energy at the penetrating height, by 9.81.

Ballistics Performance. Ballistic tests of the multi-layer panels are conducted to determine the ballistic limit (V50) in accordance with MIL-STD-662e, except in the selection of projectiles, as follows: A panel to be tested is placed against a backing material of Roma Plastina No. 1 clay in a sample mount to hold the panel taut and perpendicular to the path of test projectiles. The projectiles are 9mm full metal jacket hand-gun bullets weighing 124 grains, and are propelled from a test barrel capable of firing the projectiles at different velocities. The first firing for each panel is for a projectile velocity estimated to be the likely ballistics limit (V50). When the first firing yields a complete panel penetration, the next firing is for a projectile velocity of about 15.5 meters (50 feet) per second less in order to obtain a partial penetration of the panel. On the other hand, when the first firing yields no penetration or partial penetration, the next firing is for a velocity of about 15.2 meters (50 feet) per second more in order to obtain a complete penetration. After obtaining one partial and one complete projectile penetration, subsequent velocity increases or decreases of about 15.2 meters (50 feet) per second are used until enough firings are made to determine the ballistics limit (V50) for that panel.

The ballistics limit (V50) is calculated by finding the arithmetic mean of an equal number of at least three of the highest partial penetration impact velocities and the lowest complete penetration impact velocities, provided that there is a difference of not more than 38.1 meters (125 feet) per second between the highest and lowest individual impact velocities.

### EXAMPLES

### Preparation of layers.

Several different yarns were woven or made into layers of fabric or fibers and then made into composite structures on which to conduct stab resistance tests.
1. Plain weave fabric of 1560 denier (1733 dtex) polybenzoxazole yarn was made at 21x21 ends per inch (8.3x8.3 ends per centimeter) with an areal density of 0.47 pounds per square foot (2.3 kilograms per square meter). This yarn was available from Toyobo Co., Ltd. under the tradename of Zylon®.
2. Plain weave fabric of 400 denier (444 dtex) poly(p-phenylene terephthalamide) yarn was made at 31x31 ends per inch (12.2x12.2 ends per centimeter) with an areal density of 0.92 pounds per square foot (4.49 kilograms per square meter). This yarn was available from E. I. du Pont de Nemours and Company under the tradename of Kevlar®.
3. Plain weave fabric of 650 denier (722 dtex) polyethylene yarn was made at 35x35 ends per inch (13.8x13.8 ends per centimeter) with an areal density of 0.50 pounds per square foot (2.44 kilograms per square meter). This yarn was available from AlliedSignal, Inc. under the tradename of Spectra® 900.
4. Layers of unidirectional extended chain polyethylene fiber (UDECPE) crossplied in 0/90 degree orientation, sandwiched with polyethylene film, were used with an areal density of 0.51 pounds per square foot (2.49 kilograms per square meter). These layers were available, completely manufactured, from AlliedSignal, Inc. under the tradename of Spectra Shield Plus®

### EXAMPLE 1

Combinations of polybenzoxazole (PBO) layers with layers of the other polymers were assembled and tested for stab resistance; and the results were compared with structures of equivalent areal density made from polybenzoxazole alone or the other polymers alone. The results are set out below:

| Construction | Penetrations Energy | Areal Density | |
|---|---|---|---|
| | (joules) | (psf) | (kgsm) |
| 8 layers (PBO) plain 8.3x8.3 | 22.6 | 0.47 | 2.30 |
| | | | |
| 40 layers (PPDT) plain 12.2x12.2 | 18.1 | 0.92 | 4.49 |
| | | | |
| 12 layers (ECPE) plain 13.8x13.8 | 11.3 | 0.50 | 2.44 |
| | | | |
| 22 layers (UDECPE) | 20.3 | 0.51 | 2.49 |
| | | | |
| 8 layers (PBO) (T) 40 layers (PPDT)(B) | 67.8 | 1.39 | 6.79 |
| | | | |
| 40 layers (PPDT) (T) 8 layers (PBO) (B) | 61.0 | 1.39 | 6.79 |
| | | | |
| 8 layers (PBO) (T) 12 layers (ECPE)(B) | 76.8 | 0.97 | 4.74 |
| | | | |
| 12 layers (ECPE) (T) 8 layers (PBO) (B) | 50.8 | 0.97 | 4.74 |
| | | | |
| 8 layers (PBO) (T) 22 layers (UDEDPE) (B) | 74.6 | 0.98 | 4.78 |
| | | | |
| 22 layers (UDECPE) (T) 8 layers (PBO) (B) | 45.0 | 0.98 | 4.78 |

| | | | |
|---|---|---|---|
| (T) denotes the top or outer (knife stab) face (B) denotes the bottom or inner face | | | |

It is noted that the composite structures provide much higher penetration energy results than would be expected from a simple sum of the individual section elements of the combination. It is, also, noted that the penetration resistance is remarkably higher when the polybenzoxazole section is located on the top (exposed to the knife stab).

### EXAMPLE 2

An additional fabric was woven for use, in the Example, in combination with fabrics from the previous Example.
5. Plain weave fabric of 200 denier (222 dtex) poly(p-phenylene terephthalamide) yarn was made at 70x70 ends per inch (27.5x27.5 ends per centimeter) with an areal density of 0.26 pounds per square foot (1.26 kilograms per square meter). This yarn was available from E. I. du Pont de Nemours and Company under the tradename of Kevlar®.

Combinations of layers were assembled and tested for knife and ice pack penetration and, in two cases, ballistic resistance; and the results were compared with structures made from only a single component alone. The results are set out below:

| Construction | Areal Density (kg/m²) | Penetration Energy (joules) | | Ballistic V₅₀ (m/sec) |
|---|---|---|---|---|
| | | Knife | Ice Pick | |
| 8 layers PBO plain 8.3x8.3 | 2.30 | 22.6 | <0.5 | - |
| | | | | |
| 40 layers, 400d PPDT plain 12.2x12.2 | 4.49 | 18.1 | 0.9 | 523 |
| | | | | |
| 10 layers, 200d PPDT plain 27.5x27.5 | 1.26 | 1.8 | 20.1 | - |
| | | | | |
| 10 layers, 200d PPDT (T) 8 layers, PBO (M) 40 layers, 400d PPDT (B) | 8.05 | 68.3 | >180 | 572 |
| | | | | |
| 8 layers, PBO (T) 10 layers, 200d PPDT (M) 40 layers, 400d PPDT (B) | 8.05 | 85.0 | 80.5 | - |
| | | | | |

| Comparison | | | | |
|---|---|---|---|---|
| 40 layers, 400d PPDT (T) 8 layers, PBO (M) 10 layers, 200d PPDT (B) | 8.05 | 58.9 | 14.6 | - |

| | | | | |
|---|---|---|---|---|
| (T) denotes the top or stab face (M) denotes the middle (B) denotes the bottom or inner face | | | | |

It is noted that the composite structures provide much higher penetration energy results than would be expected from a simple sum of the individual elements of the combination. It is, also, noted that the penetration energy results are poor for the comparison composite wherein the tightly-woven layers are nearer the inner face than ballistic layers.

## Claims

1. A knife and ice pick penetration resistant article (10) comprising
a) a plurality (11) of primarily knife resistant layers (12) of woven fabric comprising polybenzoxazole or polybenzothiazole fibers and
b) a plurality (13) of primarily ice pick resistant layers (14) of tightly-woven penetration resistant fabric having a fabric tightness factor of at least 0.75.

2. The article according to Claim 1 wherein said tightly-woven penetration resistant fabric includes polyamide fibers.

3. The article according to Claim 2 wherein said polyamide fibers are para-aramid.

4. The article of Claim 1 wherein the plurality (13) of tightly-woven penetration resistant fabric layers (14) include aramid yarn having a linear density of less than 500 dtex and **characterized by** having the tightly-woven penetration resistant fabric woven to a fabric tightness factor of at least 0.95.

5. The article according to any one of Claims 1 to 4 wherein said tightly-woven penetration resistant fabric includes polyolefin fibers.

6. The article according to Claim 5 wherein said polyolefin fibers are polyethylene.

7. The article according to any one of Claims 1 to 6 wherein said tightly-woven penetration resistant fabric includes polybenzoxazole or polybenzothiazole fibers.

8. The article of Claim 1 wherein the plurality (13) of tightly-woven penetration resistant fabric layers (14) include polybenzoxazole or polybenzothiazole yarn having a linear density of less than 500 dtex and **characterised by** having the tightly-woven penetration resistant fabric woven to a fabric tightness factor of at least 0.95.

9. The article of Claim 1 wherein the fibers of polybenzoxazole or polybenzothiazole are in yarn with a linear density of 100 to 3300 dtex and the fibers have a linear density of 0.3 to 17 dtex.

## Patentansprüche

1. Ein gegen Einstiche von Messern und Eispickel resistenter Artikel (10), umfassend:
a) eine Vielzahl (11) von gegen Messer im Wesentlichen resistenten Schichten (12) aus Gewebe, umfassend Polybenzoaxol- oder Polybenzothiazolfasern und
b) eine Vielzahl (13) von gegen Eispickel im Wesentlichen resistenten Schichten (14) von dicht gewebtem gegen Einstiche resistentem Stoff mit einem Stoffdichtefaktor von mindestens 0,75.

2. Artikel nach Anspruch 1, wobei der dicht gewebte gegen Einstiche resistente Stoff Polyamidfasern enthält.

3. Artikel nach Anspruch 2, wobei die Polyamidfasern Para-Aramid sind.

4. Artikel nach Anspruch 1, wobei die Vielzahl (13) von dicht gewebten gegen Einstiche resistenten Stoffschichten (14) Aramidgarn einschliesst mit einer linearen Dichte von weniger als 500 dtex und **dadurch gekennzeichnet, dass** der dicht gewebte gegen Einstiche resistente Stoff mit einem Stoffdichtefaktor von mindestens 0,95 gewebt ist.

5. Artikel nach irgendeinem der Ansprüche 1 bis 4, wobei der dicht gewebte gegen Einstiche resistente Stoff Polyolefinfasern enthält.

6. Artikel nach Anspruch 5, wobei die Polyolefinfasern Polyethylen sind.

7. Artikel nach irgendeinem der Ansprüche 1 bis 6, wobei der dicht gewebte gegen Einstiche resistente Stoff Polybenzoxazol- oder Polybenzothiazolfasern enthält.

8. Artikel nach Anspruch 1, wobei die Vielzahl (13) von dicht gewebten gegen Einstiche resistenten Stoffschichten (14) Polybenzoxazol- oder Polybenzothiazolgarn mit einer linearen Dichte von weniger als 500 dtex enthält und **dadurch gekennzeichnet, dass** der dicht gewebte gegen Einstiche resistente Stoff mit einem Stoffdichtefaktor von mindestens 0,95 gewebt ist.

9. Artikel nach Anspruch 1, wobei die Polybenzoxazol- oder Polybenzothiazolfasern im Garn, mit einer linearen Dichte von 100 bis 3300 dtex sind und die Fasern eine lineare Dichte von 0, 3 bis 17 dtex haben.

## Revendications

1. Article résistant à la pénétration d'un couteau ou d'un piolet (10), comprenant
a. une pluralité (11) de couches essentiellement résistantes au couteau (12) en tissu comprenant des fibres de polybenzoxazole ou de polybenzothiazole et
b. une pluralité (13) de couches essentiellement résistantes au piolet (14) en tissu à tissage serré résistant à la pénétration ayant une densité de tissage d'au moins 0,75.

2. Article selon la revendication 1, dans lequel ledit tissu à tissage serré résistant à la pénétration inclut des fibres polyamide.

3. Article selon la revendication 2, dans lequel lesdites fibres polyamide sont des fibres paraaramides.

4. Article selon la revendication 1, dans lequel la pluralité (13) de couches en tissu à tissage serré et résistant à la pénétration (14) inclut du fil d'aramide ayant une densité linéaire de moins de 500 dtex et **caractérisée en ce que** le tissu à tissage serré résistant à la pénétration a un facteur de densité de tissage d'au moins 0,95.

5. Article selon l'une quelconque des revendications 1 à 4, dans lequel ledit tissu à tissage serré et résistant à la pénétration inclut des fibres de polyolefines.

6. Article selon la revendication 5, dans lequel lesdites fibres de polyolefines sont du polyéthylène.

7. Article selon l'une quelconque des revendications 1 à 6, dans lequel ledit tissu à tissage serré résistant à la pénétration inclut des fibres de polybenzoxazole ou de polybenzothiazole.

8. Article selon la revendication 1, dans lequel la pluralité (13) de couches en tissu à tissage serré et résistant à la pénétration (14) inclut un fil polybenzoxazole ou polybenzothiazole ayant une densité linéaire de moins de 500 dtex et **caractérisé en ce que** le tissu à tissage serré et résistant à la pénétration a un facteur de densité de tissage d'au moins 0,95.

9. Article selon la revendication 1, dans lequel les fibres de polybenzoxazole ou polybenzothiazole sont dans un fil avec une densité linéaire de 100 à 3300 dtex et les fibres ont une densité linéaire de 0,3 à 17 dtex.
